

## UNITED STATES PATENT OFFICE.

JOSEPH W. WEITZENKORN, OF PITTSBURGH, PENNSYLVANIA, ASSIGNOR TO MOLYBDENUM CORPORATION OF AMERICA, OF PITTSBURGH, PENNSYLVANIA, A CORPORATION OF DELAWARE.

## STEEL ALLOY.

No Drawing.

Application filed March 30, 1926. Serial No. 98,617.

In my United States Patent No. 1,287,153, there is disclosed a steel alloy containing chromium, vanadium and molybdenum, within certain percentages, the characteristic feature of the alloy being that it has great strength and ductility throughout a wide range of heat treating temperatures. Specifically, as disclosed in the patent, the high elastic limit and tensile strength of the alloy vary relatively little throughout a drawing and annealing range of temperatures of from about 500° to 1200° F. and even at the lowest of these drawing and annealing temperatures the steel is quite ductile, having a reduction of area of about 35 per cent.

The alloy so disclosed contains not more than about .60 per cent carbon, from about .50 to 1.50 per cent chromium, from about .10 to .50 per cent vanadium, and from about .50 to 1.25 per cent molybdenum, the remainder being iron with the exception of impurities and other elements customarily found in steel as a result of manufacturing processes.

My present invention relates to alloy steels such as disclosed in my said patent, and is predicated upon my discovery that an alloy steel having the same content of chromium and vanadium as that disclosed in the patent, but which contains carbon up to about 2.50 per cent and molybdenum up to about .48 per cent possesses substantially the same physical characteristics as the alloy of the patent.

The alloy provided according to this invention contains carbon up to about 2.50 per cent, from about .50 to 1.45 per cent chromium, from about .10 to .50 per cent vanadium, and molybdenum up to about .48 per cent, the remainder being iron except for the usual amounts of other elements such as sulphur, phosphorus, silicon and manganese which are ordinarily present as impurities or as incidental to manufacturing processes. The sulphur and phosphorus should be as low as possible, while silicon and manganese may be present to the extent usually found in most steels.

Within drawing and annealing temperatures of from about 500° to 1200° F., this steel alloy has very high strength, both elastic limit and ultimate, and is quite ductile even when drawn and annealed from the lowest of these temperatures.

I claim as my invention:

A steel alloy consisting of an appreciable and effective amount of carbon up to about 2.50 per cent, from about .50 to 1.45 per cent chromium, from about .10 to .50 per cent vanadium, and an appreciable and effective amount of molybdenum up to about .48 per cent, the remainder being iron except for the usual amounts of other elements present as impurities and as incidental to manufacturing processes.

In testimony whereof, I sign my name.

JOSEPH W. WEITZENKORN.